

## UNITED STATES PATENT OFFICE

2,135,327

## MOTOR FUEL CONTAINING NITRILES

Victor Conquest, Chicago, Ill., assignor to Armour and Company, Chicago, Ill., a corporation of Illinois

No Drawing. Application June 29, 1936,  
Serial No. 88,063

4 Claims. (Cl. 44—9)

This invention relates to motor fuels and it comprises a motor fuel of the hydrocarbon type, such as gasoline and kerosene containing a small amount of at least one aliphatic nitrile containing 5 six or more carbon atoms.

I have discovered that the addition to gasoline or kerosene of small amounts, of the order of 0.01 to 1 or 2 percent of aliphatic nitriles derived from higher fatty acids imparts anti-knock properties to the gasoline and also tends to prevent 10 the deposition of carbon.

All of the nitriles which I add to gasoline in accordance with the present invention are soluble in gasoline and can simply be added thereto 15 in about the amounts specified.

There are many nitriles coming within the scope of my invention. These nitriles are usually made from fatty acids by reacting the fatty acid with ammonia in the presence of a dehydrating 20 catalyst. Thus, for example, stearonitrile and palmito-nitrile are nitriles corresponding to stearic and palmitic acids. I can use nitriles prepared from capric, caprylic, lauric, myristic and stearic acids, and also prepared from the unsaturated 25 fatty acids such as oleic and linoleic. I can also use nitriles obtained by pyrolytically cracking higher fatty acid nitriles such as stearo- and palmito-nitrile. These cracked products are mostly lower molecular weight fatty acid nitriles, 30 both saturated and unsaturated, which boil from 40° C. to as high as 360° C. In many instances the cracked nitriles are associated with quantities of hydrocarbons which are also products of the cracking reaction. Methods of preparing 35 these cracked nitriles are described in Patents 2,033,536 and 2,033,537.

For example, to an ordinary cracked gasoline showing some tendency to knock, I add 0.5 percent of a mixture of nitriles obtained from cracking stearonitrile in liquid phase under pressure. 40 The exact composition of this mixture of nitriles is not clearly understood but it will contain nitriles having from six to about twelve carbon atoms. Or I can add to gasoline about 0.3 percent 45 of ordinary stearo- or palmito-nitrile. In

both instances the gasoline is improved with respect to its knocking tendency.

The lower aliphatic nitriles such as aceto-nitrile have on anti-knock properties, nor do they help in preventing the deposition of carbon in the 5 cylinders of an engine. As the molecular weight of the nitrile increases, however, I find a marked development in anti-knock properties. I have no explanation to offer for the surprising behavior of the higher aliphatic nitriles as anti-knock substances. The nitriles are rather active materials 10 chemically and possibly they aid in the combustion of fuel in some way to prevent detonation of the explosive charge in the engine.

My nitriles are also useful in the treatment of 15 kerosene to render it more suitable for internal combustion engine purposes. When treating kerosene, I find it more advantageous to add about 1 percent of the cracked nitriles or about 0.7 percent of stearonitrile. In all instances the 20 amount of nitrile present will range from a low as 0.01 percent to about 2 percent. If a motor fuel shows rather slight tendency to knock then more of the nitrile is necessary.

Of course various mixtures of nitriles each of 25 which contains at least six carbon atoms can be used and accordingly in the appended claims I use the language "an aliphatic nitrile material" to include both pure single nitriles and mixtures 30 thereof with other nitriles.

Having thus described my invention what I 35 claim is:

1. A motor fuel of the gasoline or kerosene type containing a small amount of at least one straight-chain aliphatic nitrile having at least 35 twelve carbon atoms.

2. Cracked gasoline containing a small amount of stearonitrile.

3. Cracked gasoline containing a small amount of palmitonitrile.

4. A motor fuel of the gasoline or kerosene type containing a small amount of a straight chain unsaturated fatty acid nitrile having at least 40 twelve carbon atoms.

VICTOR CONQUEST. 45